

# United States Patent Office.

JOHN D. GREY, OF PITTSBURG, PENNSYLVANIA, ASSIGNOR TO HIMSELF AND JOHN LIPPINCOTT, OF SAME PLACE.

*Letters Patent No. 95,017, dated September 21, 1869.*

## IMPROVEMENT IN THE MANUFACTURE OF GALVANIZED IRON.

*The Schedule referred to in these Letters Patent and making part of the same.*

*To all whom it may concern:*

Be it known that I, JOHN D. GREY, of Pittsburgh, in the county of Allegheny, and State of Pennsylvania, have invented a new and useful Improvement in Galvanized Iron; and I do hereby declare that the following is a full, clear, and exact description thereof, which will enable others skilled in the art to make and use the same.

The object of my invention is to provide galvanized iron of more improved quality than is now made; and

The invention consists in preparing the iron previous to galvanizing it, in a way calculated to provide a better article in point of toughness and appearance when finished, the zinc covering being disposed much more evenly and in large spangles over the entire surface of the sheet.

I am also enabled, by my improvement, to produce the same more cheaply than is now done.

Previous to describing my improved process, I will describe the common process of manufacturing it.

In the first place, the best quality of charcoal bloom-iron is generally employed, which is reduced in packs to sheets of the desired thickness between rolls, as ordinarily practised in rolling-mills, after which it is annealed in packs in a furnace, or more generally in a close iron box, placed in a furnace requiring about twenty-four hours' time.

After it has been properly annealed, the sheets are trimmed to the desired size, and are now ready for pickling in a bath prepared of water and sulphuric acid, in about the proportion of five parts of the former to one of the latter.

The object in pickling the iron is to remove the scale formed on the surface of the iron in the process of rolling it into sheets, it being absolutely necessary that all the scale shall be removed, and the surface of the iron perfectly clean, as when any scale remains it will not be covered in the process of galvanizing.

After the iron has remained in the pickle long enough to have removed the scale, which generally requires from an hour to an hour and a half, and sometimes two hours, depending upon the thickness of the scale, it is taken out and washed in water to remove or destroy the acid, after which the sheets are dipped into the sal-ammonia bath, thence into the zinc or spelter-pot for galvanizing, as commonly practised and well known in the arts.

There is a positive injury done the iron by this process of removing the scale, (which is entirely obviated by my method,) which is produced by acid penetrating the pores of the iron, when it is exposed too long in the bath, making it brittle or short in the grain, so that it is easily broken when bent.

The scales on the sheets will vary considerably in

thickness from various causes, and especially because they are rolled in packs, as they must be to obtain the necessary thinness.

The sides of the outside sheets, exposed to the action of the rolls, will have a scale very much thicker than the inside of the same sheets or the inner sheets, and this amounts to about thirty-three per cent. of the whole, as they are commonly rolled in packs of six sheets, and where it is thin, ten to fifteen minutes immersion in the acid bath or pickle is sufficient to remove it, but it is necessary to let it remain until the thick scale is also removed, so that while this is being slowly accomplished, the acid is attacking that portion of the sheet from which the thin scale was removed in the early part of the process, and eating small holes therein, and wasting away the iron.

The surface of the iron, as a natural consequence, is rough, and when it is galvanized, the zinc will not flow freely or smoothly upon it, which, in my opinion, prevents the formation of the large spangles, which are desirable.

The injurious effects of sulphuric acid upon iron, when it has been too long exposed to its influence, is well known, and while I use the acid bath or pickle in my process, the iron prepared by me has a uniform scale, or very thin oxide, all over the sheet, so that it requires but ten to fifteen minutes only to remove it, the time being so short, and the action of the acid so uniform, that no possible injury can result to the iron, which is smooth on its surface, and retains all its original toughness after it has been galvanized, the zinc having been deposited in the large spangles.

My mode of making galvanized iron is precisely the same as commonly practised, with this exception: I dispense with the annealing process, before referred to, thus saving time and expense, and so shorten the time necessary to pickle, that I am enabled to produce five times the quantity of iron cleaned, ready for galvanizing in any given time by the old process, besides running the acid bath or pickle five times as long without renewing as by the old process, which is a saving in the cost of manufacture.

To manufacture galvanized sheet-iron by my process, I take the sheets from the rolls, trim them to the required size, and dip them in a bath of muriatic acid and water, in the proportion of about one part of the former to five of the latter. After remaining a few minutes in the bath, they are taken out and set upon their edge to drain, after which they are placed in a furnace upon their edge, and held there by a rack arranged on the floor of the furnace, or by any other convenient means, care being taken that the surface of the sheet shall be exposed to the heat of the furnace, having a clear fire, as free from flame or smoke as possible.

If more than one sheet is placed in the furnace at one time, care must be taken that they in no way come in contact with each other.

The heat of the furnace being just right, in a short time the scale formed during the process of rolling will commence to raise all over the sheet, and no matter how thick it may be, the effect will be the same.

When it is judged, by the appearance of the sheet, that the scale is all loosened or raised, it is removed from the furnace, when the scales will leave the sheet in large blisters, and are swept off with a broom, so that by this process of raising the scale, by the means described, I get rid of any thick scale, and at the same time anneal the iron perfectly.

As soon as the scale commences to raise upon the sheet in the furnace, there is a new one formed beneath the old one, but it is extremely even and thin, and although necessary to remove it by the bath before galvanizing, from the fact of this thin scale being uniform upon all the iron treated by my process, there is but little delay or detention, as in ten minutes after it is placed in the acid bath or pickle the iron will be perfectly clean.

A man and a boy will scale as much as three to four tons of sheet-iron per day, and as fast as it is scaled, it is pickled and galvanized, being one continuous operation.

No one step requires essentially more time than another, and consequent delay, as in the case of annealing in the old process. Other acids or compounds, singly or in combination with water, may be used to assist scaling in a furnace.

I therefore do not limit myself to any particular material or materials to accomplish this result, the main object with me is to raise the thick and uneven scale by heat, and form a new thin one at the same time that can be easily and quickly and uniformly removed in the process of pickling, for the purpose of preventing local injury to the iron, and leave the surface smooth, so that the zinc will be deposited on it in large spangles.

Having thus described my invention, I claim as new, and desire to secure by Letters Patent—

1. The improved process, herein described, of preparing iron for galvanizing, substantially in the manner and for the purpose specified.

2. As an improved article of manufacture, galvanized iron, when prepared in the manner herein specified.

JOHN D. GREY.

Witnesses:

JOHN LIPPINCOTT,  
Jos. M. LIPPINCOTT.